

Dec. 11, 1934.

M. W. SEYMOUR

1,984,090

PHOTOGRAPHIC MATERIAL FOR MAKING COLORED PRINTS

Filed Feb. 29, 1932

BICHROMATED GELATINE LAYER CONTAINING SILVER  
IODIDE HAVING A BASIC DYE ADSORBED THERETO.



Inventor:  
*Merrill W. Seymour,*

By *Newton M. Perrine*

Attorney

## UNITED STATES PATENT OFFICE

1,984,090

PHOTOGRAPHIC MATERIAL FOR MAKING  
COLORED PRINTSMerrill W. Seymour, Rochester, N. Y., assignor to  
Eastman Kodak Company, Rochester, N. Y., a  
corporation of New York

Application February 29, 1932, Serial No. 595,971

2 Claims. (Cl. 95—7)

This invention relates to a material for making photographic prints of the type known as carbon prints and particularly to colored carbon prints.

5 The use of bichromated gelatin layers for producing photographic positives by the method called the carbon process has been known for many years. Previous workers in this process have included pigments and dyes in the 10 bichromated layers and several have introduced silver salts with or without pigments. These prior bichromated layers were sensitive however only to blue and violet light.

I have found a simple method by which a 15 bichromated gelatin layer may be optically sensitized to the longer wavelengths and at the same time contain a suitable dye for a color print. I have moreover found that a layer made according to my invention has the 20 hitherto unknown property of giving a controlled degree of contrast by simply varying the quality of the printing light.

My invention is carried out by adding to a 25 bichromated gelatin a quantity of silver iodide having a dye adsorbed to it. In practice the same result may be attained by coating a support with an emulsion containing the dyed silver iodide and then sensitizing this emulsion by bathing in bichromate. In either case the 30 result will be the same.

Reference is made to the accompanying drawing, the single figure of which shows on an exaggerated scale a section of a photographic element embodying my invention. In this figure, the support, which may be of any material 35 is indicated at 1 and this carries a layer 2 of bichromated gelatin containing silver iodide having basic dyes strongly adsorbed thereto.

The method of making and the character 40 of these materials are more fully described hereinafter.

As a specific example plates may be prepared from the following formula:

## I

45 Gelatin, 12.5% solution..... 40 c. c.  
Water..... 30 c. c.  
Turquoise blue G, 1%..... 20 c. c.  
Silver nitrate, 10%..... 15 c. c.

## II

Potassium iodide, 10%..... 18 c. c.  
Water..... 22 c. c.  
II is slowly poured into I while the mixture is 50 stirred. The resulting emulsion is set, shredded,

and washed for  $\frac{1}{2}$  hour in cold-running water. 5 10 c. c. of the remelted washed emulsion coated on a 5in.  $\times$  7in. plate will provide a satisfactory example. A transparent blue-green coating will be obtained by this procedure. A plate thus coated is now bathed 5 minutes in the following solution and dried:

Ammonium bichromate..... 25 grams  
Ammonia solution concentrated..... 5 c. c.  
Water to..... 1 liter 10

If portions of this sensitized plate are exposed through the glass side behind the same negative for, say, three minutes to a 5-ampere arc lamp at one foot for one portion and three 15 minutes to a 500-watt tungsten filament lamp at one foot for the other portion, it will be found after development that the print made with Tungsten lamp is somewhat denser than the other. This is of course contrary to the behavior 20 of the older bichromated layers and shows a marked increase in the sensitivity of the layer for the longer wavelengths. It is understood of course that these prints are developed, as for the usual bichromated prints, in 25 water at about 110° F., producing transparent blue-green relief images with the particular dye mentioned in the example.

The sensitivity of the bichromated gelatin to 30 all portions of the visible spectrum may be readily shown by exposing to light through suitable filters. The following experiment will illustrate. A plate sensitized as above was exposed through the glass side behind the series of neutral densities ascending in uniform steps of 0.2 and covered 35 in different portions by Wratten filters 29 (red), 61 (green), and 49 (blue). Exposure was for 12 minutes to arc lamp at one foot and a print was developed in water at 110° F. The relief image of blue-green color was obtained 40 showing five steps for the red filter, three steps for the green filter and five steps for the blue filter. The sensitivity of the bichromated gelatin to all portions of the visible spectrum is thus clearly indicated. 45

In this experiment the contrast of image was very high through the green filter, but moderate through the red and blue filters. The contrast is therefore reduced in those regions in which the emulsion absorbs light most strongly. With 50 the plates described, the dye absorbs strongly in the red region and to some extent, probably, in the violet. The silver iodide absorbs strongly in the violet region. Neither substance absorbs to so great an extent in the green region. 55

It is therefore apparent that the method I have just described may be made the basis of a means for controlling the contrast of a carbon print in a manner which has not heretofore been possible.

This may be done by varying the spectral quality or color of the printing light so as to attain either a high contrast or a lower degree of contrast. If a high contrast is required, one prints 10 the bichromated layer sensitized as described by light from a region only slightly absorbed by the emulsion. By admitting a lesser amount of light of this color and admitting more of the light which is more strongly absorbed by the emulsion 15 (complementary in color) the contrast is reduced. To secure the minimum contrast one would print entirely to light of the color complementary to the emulsion. In the example described, a red filter would be indicated, for 20 example.

I propose to apply the above method of carbon printing to the making of prints from black and white negatives and making color prints from color separation negatives or directly from color 25 negatives on screen plates or direct subtractive color plates. My invention offers marked advantages for the well-known method of making superposed color transparencies.

As an example of making a color print from 30 an autochrome negative, I first make a print from a negative on to a blue-green emulsion of the kind described using a red filter. I then make a print on to a magenta emulsion using a green filter and on to a yellow using a blue 35 filter. The three prints, having been developed in warm water and dried are superposed in register to form a color positive which may be either a transparency or a paper print.

A large number of dyes, particularly basic dyes, are available for use to yield a large variety of colors. In fact, I have found that many, if not most, basic dyes that are strongly colored and are strongly adsorbed to silver iodide are 5 operative, even though they are not in themselves sensitizers for silver halides in the ordinary photographic process involving a brief exposure to light and a subsequent development of a silver image by means of an alkaline reducing solution. These dyes, of course, vary 10 widely in their efficiency but the operative dyes for this purpose are so numerous and well known that it would be almost impossible to give a complete list. While I have illustrated my invention with a single dye and a single formula, it is of course understood that my invention is not limited to that particular form described. It will be apparent that a large number of variations and modifications in the procedure may be 15 20 made, all of which I consider as included in my invention as expressed by the appended claims.

What I claim is:

1. A permanently colored light-sensitive layer 25 for use in carbon printing and comprising gelatine, an alkali bichromate and silver iodide having adsorbed thereto a basic dye having the characteristics that it is strongly colored, that it is strongly adsorbed to the silver iodide and is permanently retained in the developed relief 30 image and that it extends the color sensitivity of the layer to all colors of the visible spectrum.

2. A permanently colored light-sensitive layer comprising bichromated gelatine and silver iodide having adsorbed thereto a strongly colored basic dye which is permanently retained in 35 the developed relief image.

MERRILL W. SEYMOUR.